

Jan. 29, 1929.

1,700,288

G. S. FULCHER

METHOD OF MAKING SOLID CAST REFRACTORY ARTICLES

Filed Oct. 18, 1927

*Fig. 1.*



*Fig. 2.*



*Fig. 4.*



*Fig. 3.*



INVENTOR

Gordon S. Fulcher.

BY

*Drey S. Cole.*

ATTORNEYS.

## UNITED STATES PATENT OFFICE.

GORDON S. FULCHER, OF CORNING, NEW YORK, ASSIGNOR TO CORNING GLASS WORKS,  
OF CORNING, NEW YORK, A CORPORATION OF NEW YORK.

## METHOD OF MAKING SOLID CAST REFRACtORY ARTICLES.

Application filed October 18, 1927. Serial No. 226,986.

This invention relates to improvements in refractories, and more particularly to the manufacture of solid cast refractory articles free from internal flaws or voids.

5 Cast refractory articles of the character to which this invention relates are produced by subjecting raw materials, such as ores consisting largely of lumina, silica, zirconia and the like, to high temperatures, whereby 10 they become fused and melted together, after which they are poured into molds of suitable shapes and sizes, and annealed. Due to the great difference in volume between the liquid and solid states of these 15 materials, the shrinkage which takes place upon their solidification creates voids or cavities in the finished product. These are commonly known in the art as "pipe" and are objectionable as they increase the rapid- 20 ity of deterioration of the article and consequently reduce its period of utility. Furthermore, such pipe lightens the casting and may make the specific gravity of the article less than that of the material in connec- 25 tion with which it is used. This is particularly true when the refractory is used to line glass melting tanks as it may give the article a tendency to float away from its predetermined position in the liquid glass, especially 30 if the tank is provided with exterior insulation. Thus the stability of the article and, under certain circumstances, its utility may be affected.

It is an object of the present invention 35 to produce a cast refractory article which will be free from such pipe and the consequent disadvantages above set forth.

A feature of the invention is the second 40 pouring of the refractory material prior to the complete solidification of the material of the first pouring, whereby the pipe formed in the material of the first pouring by the solidification of a portion thereof is filled, and the refractory material used in 45 the second pouring unites with that of the first pouring to form a homogeneous mass.

The above and other objects are attained by practicing the method constituting the subject matter of the present invention,

which will be fully set forth and claimed in 50 the following specification, and illustrated in the accompanying drawing, in which:

Fig. 1 is a longitudinal, sectional view through a mold and casting illustrating the formation of the pipe within the casting 55 upon completion of the first pouring;

Fig. 2 is a similar view illustrating the mold prepared for the second pouring;

Fig. 3 is a similar view showing the mold upon completion of the second pouring and 60 after the complete solidification of the liquid forming the article; and

Fig. 4 is a perspective view, on a reduced scale, of a finished block made by the invention set forth herein. 65

Referring to the drawings, 10 designates a mold of any suitable substance and configuration but, for the purpose of illustrating my invention, it is shown as constructed to form a cast refractory block of the type 70 used to line glass melting tanks or the like. The mold includes bottom, side and end walls 11, formed of sand bonded together by linseed oil and baked to produce slabs, which are connected in any suitable way, 75 as by cementing them together along adjacent edges to form a box. A top slab 12 is secured to the upper edges of the side and end walls 11, and is provided with a central opening or gate 13 through which the refractory material is poured. 80

The mold is placed within a container 14, of metal or other suitable substance, and is supported in spaced relation to the bottom of the container by suitable heat insulating 85 bricks 15. A slab 11' may be interposed between the bricks and the mold bottom but is not absolutely essential to the herein-described invention. Resting upon the top slab 12 of the mold is a slab 16, provided with a central opening 17 arranged to register with the opening 13 in slab 12. To

properly space the mold 10 from the sides of container 14, and to prevent the slabs 11 from bulging during or after the pouring operation, insulating bricks 18 are arranged in spaced relation to each other at 90 the sides of the mold. The interstices be-

tween the bricks are filled with a suitable heat insulating material 19, such as silocel.

Supported on the slab 16 is a font mold 20 which, in the present instance, has a tapered cylindrical body of cast iron or the like. The reduced end of said font mold is disposed upwardly, so that it may be readily removed from the font after the pouring has taken place. The space between the font mold and the walls of the container 14 is filled with the insulating material 19 to completely insulate the mold and to prevent too rapid cooling of the casting.

15 When it is desired to cast an article the mold, prepared as above described, is placed in position to receive the molten refractory, which is then poured into the mold through the font mold 20. The molten refractory is poured to a height about three inches above the lower end of the font mold, as shown in Fig. 1, and due to the shrinkage of the material, while solidifying, the font will become exhausted of molten material 25 thus forming a pipe or void 21 within the casting.

Before the casting has completely solidified, the insulating material between the font mold 20 and the container is removed, together with the font mold, and the font 30 22, formed by the setting of the molten material at the lower end of the font mold, is broken away to expose the pipe, as shown in Fig. 2. A new cover slab 12' is then placed on the casting and the font mold is replaced, whereupon a second pouring is effected, as shown in Fig. 3, so that the pipe becomes completely filled and the casting is thus made solid. The second pouring takes 35 place within a reasonably short time after the first pouring, that is before the liquid of the first pouring has completely solidified, so that the material of the second pouring will unite with that of the first pouring, and 40 form a homogeneous mass. In the second pouring the font mold 20 is nearly filled with the molten refractory material to insure a sufficient supply of the molten material to 45 fill the pipe.

50 When the outside of the second font 23 has set, the font mold is removed and the font is surrounded with insulating material. After complete solidification of the cast article 24, the font 23 is broken away and 55 any scar 25 formed thereby is smoothed to remove objectionable projections. The casting is then covered with heat insulating material and set aside to anneal, as explained in detail in Patent 1,615,750, issued to me 60 on January 25, 1927. After annealing the casting is removed and, if so desired, any or all of the surfaces thereof may be ground smooth and trued.

There are instances when a large scar,

such as 25, may prove objectionable and, 65 since the size of the scar is determined by the diameter of the gate, it may be found desirable to use a relatively small gate, and thus necessitate the use of a plurality of fonts in succession to supply liquid until the 70 casting has completely solidified.

Due to the rapidity of solidification of the molten refractory material, and its tendency to produce a uniform external crust about the casting, upon contact with the 75 cooler mold surfaces, articles having a greater depth than the size of the gate opening cannot be poured free from pipe with a single pouring, as the material will solidify and close the gate, thus preventing 80 the molten material in the font from entering the mold as shrinkage of the contents thereof takes place. Thus the use of a plurality of fonts in succession, as just described, must be resorted to when the thickness 85 of the casting exceeds the diameter of the largest gate which can be used in producing it. Solid cast articles free from pipe can be produced with a single pouring if the thickness of the casting is less than the 90 diameter of the permissible gate.

Thus it will be seen that, by practicing the method herein described, refractory articles of any thickness may be cast solid and free from voids and similar imperfections.

While in the foregoing there has been shown and described the preferred embodiment of this invention, it is to be understood that various modifications in the details of 100 procedure, as well as in the apparatus used, may be resorted to within the scope of the following claims.

I claim:

1. The method of making solid cast refractory articles which includes pouring molten refractory material into a mold, allowing a portion of said material to solidify and shrink, and feeding additional molten refractory material into the mold to compensate for the shrinkage of the material first poured.

2. The method of making solid cast refractory articles which includes pouring molten refractory material into a mold, 115 forming a font of the refractory material to supply additional material to the mold as the material therein solidifies and shrinks, breaking away the font, and pouring additional material into the mold.

3. The method of making solid cast refractory articles which includes pouring molten refractory material into a mold, forming a font of the refractory material to supply material to the mold as the contents 125 thereof solidify and shrink, breaking the font away from the article, pouring additional material into the mold to compen-

sate for other shrinkage of the material, and annealing the article.

4. The method of making solid cast refractory articles which includes pouring molten refractory material into a mold, forming a font of the refractory material to supply additional material to the mold as

the contents thereof solidify and shrink, breaking said font away after it has become exhausted of molten refractory material, and 10 forming other fonts of the refractory material to supply still further material to the mold as its contents solidify and shrink.

GORDON S. FULCHER.